

May 19, 1931.

W. A. MUDGE ET AL

1,806,408

TRANSFORMER

Filed Oct. 2, 1928

| Metal or Alloy.       | Flux Density<br>H-100Gausses. | Saturation<br>Value<br>(Gausses) | Values from<br>Bureau of<br>Standards<br>Circular #100.<br>Page 93. |
|-----------------------|-------------------------------|----------------------------------|---------------------------------------------------------------------|
| Pure Iron             | 18,500                        | 22,500                           |                                                                     |
| 50% Iron-Nickel Alloy | 15,500                        | 15,500                           |                                                                     |
| Pure Nickel           | 6,000                         | 6,000                            |                                                                     |
| Monel Metal           | 2,200                         | 2,200                            |                                                                     |

Fig. 1



Fig. 2

INVENTORS  
William Alvin Mudge  
Clarence George Biber  
by their attorney  
Henry Stetlin - Pameke.

## UNITED STATES PATENT OFFICE

WILLIAM ALVIN MUDGE AND CLARENCE GEORGE BIEBER, OF HUNTINGTON, WEST VIRGINIA

## TRANSFORMER

Application filed October 2, 1928. Serial No. 309,843.

This invention relates to an improvement in alternating current transformers, and relates particularly to low power transformers, i. e., transformers whose power output is not substantially in excess of five hundred watts, and preferably lower. 55

Low power transformers are required in a great many different kinds of electrical appliances. They are used for instance in supplying the cathode voltage to alternating current radio tubes, radio sets employing rectified and filtered alternating current, electric clocks run by small motors, and other apparatus. As generally constructed, a fluctuation in the primary voltage, such as the fluctuation that occurs in the usual commercial one hundred ten volt line causes a corresponding fluctuation in the secondary or output circuit of the transformer. This non-uniform output of the transformer is undesirable in most types of work for which such transformers are intended. Most devices employing a low power transformer require a constant source of energy for their operation. 65

Heretofore a ballast lamp in series with the primary circuit or other regulator has been employed for eliminating fluctuations in the output of the transformer.

According to the present invention we provide a low power transformer for producing and maintaining a constant energy output independent of the normal fluctuation in the supply or primary voltage. 75

It is well understood by those skilled in the art that a transformer is an electrical device having two electric circuits, a primary and a secondary linked by a common magnetic circuit formed by the core of the transformer. The amount of energy which can be transferred from the primary to the secondary through the core is limited by the magnetic saturation value of the core material. When a transformer is loaded so that the core of the transformer is working at or near its saturation point, an increase in the voltage impressed across the core of the transformer produces no further appreciable increase in the energy which the core carries across to the secondary of the trans- 85

former. If the core of the transformer is not working at or near its saturation point, increases in the voltage across the primary result in corresponding increases in the energy carried by the core to the secondary of the transformer with a consequent variation in the output of the secondary. This variation or fluctuation is not desirable. 95

A small transformer should have a rather high primary inductance (about three to five henries at 110 volts) in order to limit the no-load current to a value small enough so that the primary winding will not dangerously overheat and to avoid a high energy waste. 100

According to our invention the transformer is designed to operate at or near the saturation point of the core material. The saturation point for certain well known core materials is shown in the accompanying drawing showing typical B—H curves for various well known materials, together with a chart of the saturation values of certain metals with their corresponding flux densities. 110

With reference to the drawing, it may be stated that the B—H curve for any magnetic material shows the relationship between the magnetic induction and the magnetizing force producing that induction, the B value being rated in gauss and the H value being gilberts per centimeter. Permeability is the relationship of B to H, and the point of saturation is the highest point of the curve. 120

In order to operate at or near the saturation point of the core material in a small transformer, it is possible to use either a very small amount (1 to 3 ounces) of silicon steel, or one of the usual core materials having a very high saturation value, or a moderate amount (1 to 10 pounds) of a material having a much lower saturation value. The use of a very small amount of material having a high saturation value for constant energy output is objectionable because of the fact that it is necessary to use a large number of primary turns in order to secure a sufficiently high primary impedance. 130

Therefore, according to the present invention, we use a core material not generally 140

considered desirable for transformer purposes. We use a core material having both high permeability and a low saturation point. By choosing a core material having both high 5 permeability and low saturation, it is easy to obtain a high primary impedance without the use of an excessively great number of turns in the primary winding. At the same time, the low saturation value of the material 10 makes it possible to operate near the saturation point of the core even though the transformer is delivering only a few watts.

In the accompanying drawing it will be seen that annealed sheet Monel metal has a 15 low saturation value, its saturation value not exceeding approximately twenty-two hundred gausses. Nickel has a saturation value of approximately six thousand gausses. Both Monel metal and nickel are therefore not 20 metals which would ordinarily be considered desirable for transformer core purposes. According to the present invention we prefer to use a metal containing nickel in a large proportion wherein the saturation value is 25 relatively low.

The saturation value of nickel and nickel alloys, such as Monel metal, is very low as compared with some well known transformer core materials. Pure iron, for instance, has a saturation value of approximately twenty-two thousand gausses. Some 30 alloys of iron and cobalt have even higher saturation values. The saturation value for silicon steel is approximately twenty-one thousand; nineteen thousand for silicon contents of one 1-4.5%. Permalloy, on the other 35 hand, has a relatively low saturation value approximately ten thousand gausses.

According to our invention, typical core 40 materials having desirable characteristics may be grouped as follows:

1. Copper-nickel alloys—containing 60-90% nickel, 10-40% copper, trace-5% manganese, trace-10% iron, trace-2% silicon and 45 none-.25% carbon. Monel metal, which contains approximately 68% nickel, 29% copper, 1% manganese and 2% iron, together with small amounts of carbon and silicon, is a commercial alloy of this type.

2. Iron-nickel alloys—containing more 50 than 30% nickel and less than 70% iron with small amounts of carbon, silicon and manganese. Permalloy, which contains 80% nickel, and 20% iron is a commercial alloy of 55 this type.

3. Nickel, containing not less than 95% nickel with 5% of cobalt, iron, manganese, copper, silicon and carbon. Commercially 60 pure nickel containing 99% of nickel is a commercial material of this type.

By using a core material in a transformer containing one of the above alloys, or other metal having similar saturation values in relation to the permeability, the transformer 65 has both a sufficiently high primary imped-

ance to avoid dangerous overheating, together with a core capable of carrying only a predetermined amount of energy to the secondary. Hence the secondary delivers a constant amount of energy independent of the fluctuations and variations in the primary voltage or impressed E. M. F., and this is so even though the output of the secondary is of an extremely low order.

Such a transformer is particularly adapted 70 to the operation of various devices requiring a low power constant source of energy for their operation, and is both cheaper and more durable than the transformer heretofore provided for such purposes wherein the transformer is used with a ballast lamp or other more complicated voltage regulator.

We claim:

A transformer having a core composed at 75 least in part of Monel metal.

In testimony whereof we have hereunto set 80 our hands.

WILLIAM ALVIN MUDGE.  
CLARENCE GEORGE BIEBER.

90

95

100

105

110

115

120

125

130